

## UNITED STATES PATENT OFFICE

2,614,986

GREASES BASED ON FINELY DIVIDED  
INORGANIC MATERIAL

Alan Beerbower, Baltimore, Md., and Arnold J. Morway, Clark, N. J., assignors to Standard Oil Development Company, a corporation of Delaware

No Drawing. Application November 12, 1948,  
Serial No. 59,748

5 Claims. (Cl. 252—25)

1

The present invention relates to greases thickened with finely divided inorganic materials, and, in particular, to lubricating greases having high melting points prepared from lubricating oil and light colored finely divided inorganic materials such as magnesium oxides and carbonates.

In the prior art, lubricating greases have ordinarily been composed of a soap-thickened oil, particularly a mineral base lubricating oil, thickened to a pasty or solid consistency with about 3 to 25% or more of metal soaps of fatty materials. Soaps such as calcium stearate, sodium stearate, and like compositions, prepared from fatty acids and/or vegetable or animal fats, have ordinarily been considered the most suitable thickening materials for lubricating greases. By their use, lubricating oils of a chosen consistency or viscosity may be gelled or solidified so that the lubricant may remain in place and not run or leak away from the point where lubrication is desired. The lubricating properties are determined in large measure by the grade, viscosity, etc., of the oil, the filler or thickener serving mainly to solidify the material and keep the oil available at the point of lubrication to carry out its intended function.

Instead of soap thickeners, various substitutes have recently been developed which have certain desirable features for such uses. Thus, greases have been prepared from lubricating oils and carbon black of high oil absorptivity or so-called high structure index. The reticulated or chain-like particled carbon blacks such as acetylene black have been found in the prior art to be excellent materials for this purpose.

Other inorganic materials such as bentonite and silica gels have been proposed as the thickening agents for lubricating oils. Some of these are unduly abrasive and, therefore, not very satisfactory, and others, such as the carbon blacks, are objectionable from the standpoint of workmen because of their extreme blackness and tendency to stain hands and clothing excessively. In addition, there are numerous instances where a light colored grease is preferred, for example, where grease is likely to drip and discolor material being worked on or where it is desirable to be able to observe the functioning of lubricating parts which would be obscured by a black or highly colored grease.

It is, therefore, an object of the present invention to prepare a lubricating grease of light color, approaching the color of the oil and having either a good degree of transparency or a light color approaching white. Certain inorganic sub-

2

stances, of which the oxides and carbonates of magnesium are particularly desirable, have the light colored characteristics desired and according to the present invention are found to be suitable grease-thickening agents. They are extremely porous and hence have high oil absorptivity. They are finely subdivided in structure so as to be quite free of abrasive properties and they possess the property of thickening lubricating oils to grease consistencies in reasonably small concentrations. They may be used either with mineral base lubricating oils or with synthetic oils such as esters of dibasic acids, polyalcohol oils, silicone polymer oils, and the like. These inorganic compounds are not used as saponifying agents in the present case, but are used as unneutralized thickeners.

The substantially unneutralized oxides and carbonates of magnesium appear to be particularly suitable for the purposes of the present invention because of the peculiar position of magnesium in the periodic table. Magnesium is the transition element between relatively alkaline and relatively amphoteric elements of the alkaline earth group. Calcium and zinc oxides, which are below magnesium in this group, have been used in greases, but magnesium oxide appears to be much superior to either in its capacity to hold oil, and hence in its grease thickening capacity. Proportions of 10 to 25%, by weight for example, of magnesium oxide or carbonate, thicken oils effectively to grease consistencies, whereas proportions of as much as 50 to 60% of either the zinc or the calcium oxides or carbonates are required for similar thickening or grease forming effect.

The magnesium compounds further appear to have outstanding properties in being lubricants of themselves, whereas the corresponding calcium compounds are too abrasive and also too reactive chemically for lubricating metal bearings. It should be emphasized that the magnesium oxides and carbonates used in the present invention are not neutralized with fats or fatty acids. They are to be distinguished, therefore, from compositions which include magnesium soaps of fatty or other saponifiable materials.

In general, a grease of the type to which this invention relates consists of a suitable lubricating oil having a viscosity which may be as low as 35 S. S. U. at 100° F. or as high as 1,000 S. S. U. at the same temperature. The oils may have any suitable viscosity index, but in view of the fact that the greases in question are particularly suitable for high temperature use, oils of fair-

ly high viscosity index may be preferred. The concentrations of the inorganic material may vary rather widely from as little as about 5% to as much as about 40% by weight, based on the finished lubricant. A grease of the general consistency of NLGI grade #2 may be prepared by adding 15 to 20% of either unneutralized MgO or MgCO<sub>3</sub>. The preferred range is usually between 10 and 25% of the filler material. Greases of other consistencies can be prepared by varying the amount of filler or thickener and also to some extent by the choice of lubricating oil. In general, the term "grease" in this specification is intended to refer to a solid lubricant of true colloidal or gel-like character, that is, a composition having an ASTM penetration, when worked, of less than 390 mm./10. Usually a still lower penetration number is obtained. The compositions of this invention thus are not to be confused with liquid lubricants which contain mere suspensions of inorganic materials. The invention will be more fully understood by reference to the following specific example.

*Example*

A lubricating grease was prepared by milling together 18% by weight of a light oxide such as Baker's light magnesium oxide and a Colombian distillate of 300 S. S. U. viscosity at 100° F. (50 at 210° F.). The oil was added slowly to the oxide while milling proceeded. The resulting grease showed a worked penetration of 243 mm./10 by the ASTM test method. The lubricant was tested by running it in the Shell Four Ball Machine and was found to produce less wear than several compounded mineral oils containing a polybutene thickener commonly used to impart tacky or adhesive properties to greases. The material prepared was also run in the A. B. E. C. machine for 24 hours at 3500 R. P. M. No noticeable wear was found in the 204 8-ball single race bearing which was used in this test or separation of oil from the inorganic thickener. The melting point of the grease was considerably above 500° F. and was in fact above the evaporation point of the oil used.

Other magnesium oxides which are available commercially were tested in the same manner as that described in the example. It was found that the very light materials were most satisfactory, those having bulk densities of more than about 2 lbs./gallon being somewhat unsatisfactory in that excessive amounts were required to obtain a desired grease consistency or hardness. Various magnesium carbonates were also tested and these followed the same general rule. Greases prepared from the lighter magnesium carbonates appeared to be slightly superior to those prepared from the oxides. The choice between using magnesium oxide and magnesium carbonate may depend in part upon the desired alkalinity of the finished product. The oxides, of course, are more highly alkaline and for this reason greases prepared from them may be considered undesirable for some uses. Such alkalinity can be overcome, at least in part, by

partially neutralizing the oxides, as by adding moderate amounts of fatty acids but these of course result in the production of soaps which are likely to have fairly low melting points and to render the grease less satisfactory for high temperature use if appreciable quantities of soaps are present.

The carbonates are more nearly neutral, although they may also react with saponifiable materials to produce some soap products. Where alkalinity is objectionable, the carbonates usually may be found to be superior.

It will be understood that the compositions of this invention may comprise from 60 to about 95% by weight of a suitable lubricating oil which may be a mineral base oil or a synthetic oil, together with as much as 40% to as little as 5% of the thickener, based on the weight of the finished product. The narrower ranges of 10 to 25% are usually preferred, calculated on the basis of the unneutralized inorganic material. The base oils may contain various modifiers such as anti-oxidants, extreme pressure compounds, tackiness agents, viscosity index improvers, rust inhibitors, sludge or corrosion inhibitors, and the like. They may be added to the finished grease rather than being added to the oil as desired, as is well understood in the art.

What is claimed is:

- 30 1. A solid grease composition consisting essentially of a mineral base lubricating oil of 35 to 1000 S. S. U. viscosity at 100° F. thickened to a grease consistency with 10 to 25% by weight of a finely divided inorganic material having a bulk density of less than 2 lbs./gallon in its normal finely divided dry condition, said inorganic material being selected from the group consisting of magnesium oxide and magnesium carbonate.
- 40 2. A composition as in claim 1 wherein the thickening agent is magnesium oxide.
- 35 3. A composition as in claim 1 wherein the thickening agent is magnesium carbonate.
- 45 4. A solid lubricating grease comprising a mineral base lubricating oil of 35 to 1000 viscosity at 100° F. containing 10 to 25% by weight, based on the total composition, of finely divided magnesium oxide.
- 50 5. Composition as in claim 4 wherein said magnesium oxide comprises about 18% of the weight of the total composition.

ALAN BEERBOWER.  
ARNOLD J. MORWAY.

REFERENCES CITED

The following references are of record in the file of this patent:

UNITED STATES PATENTS

| Number     | Name        | Date          |
|------------|-------------|---------------|
| Re. 16,943 | Judd        | Apr. 24, 1928 |
| 650,108    | Holm        | May 22, 1900  |
| 1,015,920  | Winkler     | Jan. 30, 1912 |
| 1,253,362  | Farkas      | Jan. 15, 1918 |
| 1,913,953  | Prendergast | Jan. 13, 1933 |
| 2,234,367  | Chesny      | Mar. 11, 1941 |